

May 27, 1941.

J. BJORKSTEN ET AL

2,243,078

TRANSFER SHEET AND COMPOSITION FOR PRODUCING REINKABLE IMPRESSIONS

Filed Feb. 4, 1938

Fig. 1.



Fig. 2.



Inventors:  
Johan Bjorksten,  
William F. Champion  
By: *J. Bjorksten, W. F. Champion*  
Zabel, Carlson, Gutlaugh & Wells  
Attorneys

Patented May 27, 1941

2,243,078

# UNITED STATES PATENT OFFICE

2,243,078

## TRANSFER SHEET AND COMPOSITION FOR PRODUCING REINKABLE IMPRESSIONS

Johan Bjorksten, Chicago, and William J. Champion, La Grange, Ill., assignors to Ditto, Incorporated, Chicago, Ill., a corporation of West Virginia

Application February 4, 1938, Serial No. 188,706

6 Claims. (Cl. 41—41.5)

This invention relates to improvements in transfer media and more particularly to improvements in transfer sheets suitable for use in a typewriter which will give impressions on a contacting sheet which may be re-inked. The invention includes transfer compositions per se.

Transfer sheets which may be used in a typewriter to create impressions on a contacting sheet which are capable of absorbing ink or color material contain an oily or oleaginous material. When an oily or oleaginous material is used alone or solely with pigments or dyes, the impressions, while capable of absorbing color to some extent, are not capable of being re-inked many times without wearing off. Copy sheets contacted with the inked impressions therefore soon become smeared and the transferred impression becomes indistinct, after only a few copies have been obtained.

An object of this invention is to provide a transfer sheet which when used in a typewriter in the manner of ordinary carbon paper, will give impressions on a master sheet of an ink-absorbing material of such permanency that these impressions may be inked, contacted directly with copy sheets, and re-inked thousands of times without wearing off.

Another object of this invention is to provide an ink absorbent composition which when coated on a thin, flexible sheet material will be transferable by pressure or impact to a sheet and yet be highly adherent to the sheet, including non-fibrous sheets such as thin aluminum plates.

Other objects and features of this invention will become apparent as the following detailed description progresses, reference being had to the accompanying drawing, in which

Fig. 1 is a perspective view illustrating assembly of the transfer sheet and master copy in a typewriter to produce negative impressions.

Fig. 2 is a perspective view illustrating the printing of positive copies from the master copy.

In accordance with the invention a thin sheet suitable for use in a typewriter is coated with a composition comprising a mixture of an oily or waxy color binding material and a compatible resin adhesion securing agent, the proportion of oleaginous material and resin being such as to form a composition which will be transferable to a contacting sheet material by the impact of the keys of a typewriter, the pressure of a pencil or the like, as will ordinary carbon paper.

The suitable color binding agents are oily or waxy materials which are water repellent and ab-

5 sorbent of color material. In general, these color binding agents are of liquid or smeary nature, and have little adhesive power. The preferred color binding agents for most color inks are soya bean oil, and paraffin oil. Other good color binding agents are oleic acid, undecylenic acid, and castor oil. Cedarwood oil, rape seed oil, and olive oil are operative. Solid or semi-solid oleaginous materials such as petrolatum, paraffin wax, lauric or myristic acid, and the like may also be used as color binding agents.

10 The suitable adhesion securing agents are resins which are compatible with oleaginous materials and have adhesive qualities greater than oleaginous materials.

15 The most suitable resins are the hydrocarbon resins obtained by the polymerization of unsaturated hydrocarbons. Resins of this type which have given superior results are the resins sold by the Monsanto Chemical Co. at the time of filing this application under the trade name of "Santo resins." These Santo resins are obtained by the treatment of cracked petroleum distillates with anhydrous aluminum chloride and similar Friedel-Crafts catalysts. The method of obtaining these resins and their characteristics are described in numerous patents, for example that granted to Charles A. Thomas and Carroll A. Hochwalt, No. 1,836,629, issued December 15, 1931. Briefly, the described process consists in agitating petroleum products of unsaturated character, such as, for example, may be obtained by cracking processes, with a small proportion of anhydrous aluminum chloride for a short period of time, whereby resin is formed by polymerization. The aluminum chloride is subsequently removed and the soluble resin is recovered from the solution by distillation or evaporation.

20 40 Cumar DX—the trade name of a paracoumarone-indene (melting range 75—85° C.) manufactured by Barrett Co. A dark brown opaque solid resin.

25 45 Cumar RS—the trade name of a paracoumarone-indene (melting range 45—55° C.) manufactured by Barrett Co. A dark reddish viscous mass.

Neville R-10 Hard—the trade name of coumarone-indene type (melting range 130—150° C.) manufactured by Neville Co. Clear amber, hard, brittle resin.

30 50 Neville R-15 Medium—the trade name of coumarone-indene type (melting range 100—130° C.) manufactured by Neville Co. Clear amber, hard, brittle resin.

In one embodiment of this invention the coating of the transfer sheet contains additional substances whose purpose is mainly to improve the mechanical characteristics of the transfer composition but which also may be color binding agents, although in general they will not be as good color binding agents as soya bean oil, oleic acid, and other liquid oily materials. These additional materials are generally solid or semi-solid, of a waxy nature, which are miscible with the fluid color binding agents and the resinous adhesive securing agents. The type and amount of these materials is chosen so as to improve the mechanical characteristics of the composition over what can be obtained in general by the use solely of ink-binding agents such as soya bean oil and the adhesive resins. Thus the fluidity and melting point of the transfer composition can be increased by the addition of such waxy or greasy materials as for example paraffin wax, carnauba wax, candelilla wax, hydrogenated castor oil, hydrogenated olive oil and the like.

In another improved form of the invention stabilizers which are primarily anti-oxidants are added to the transfer composition. Such materials as inhibitol, hydroquinone and naphthols are useful in retarding the oxidation of oils such as soya bean oil.

Dyes which are compatible with the resins and 30

very intimately with a liquid wax, they will not be greatly detrimental.

The proportion of the various ingredients in the transfer composition may be varied widely.

5 The adhesive resin may vary from about 1% to about 75% by weight on the basis of resins plus oleaginous and waxy materials. The most suitable proportions, however, will vary according to the type of resin, its compatibility with the

10 oily and waxy materials, and its adhesive power. The resin should not be present in such amount that it will prevent the transfer of the composition by pressure or impact. In the case of Santo resins the preferred proportion will vary from

15 about 10% to 50% by weight on the basis of the resin plus oleaginous material. In most cases these proportions approximately correspond with the per cent on the basis of the entire transfer composition, since the anti-oxidants and dyes, if present at all, will be present in small amount, as

20 1% or less.

25 The following formulae given in Table I will serve as examples of compositions which, when applied to base materials such as tissue paper or the like by methods known to the art, form sheets yielding impressions of greatly enhanced adhesive properties. If production of a dye-carrying sheet is desired, the dyes may be incorporated in these compositions by means well known to the art.

TABLE I  
*Percentage composition*

|                                        | 1  | 2  | 3  | 4  | 5  | 6  | 7  | 8  | 9  | 10 | 11 | 12 |
|----------------------------------------|----|----|----|----|----|----|----|----|----|----|----|----|
| Soya bean oil.....                     | 25 |    |    |    | 15 | 20 |    | 15 |    | 15 |    |    |
| Undecylenic acid.....                  |    | 30 |    |    | 15 |    | 10 |    |    |    |    |    |
| Castor oil.....                        |    |    | 25 |    |    |    | 10 |    | 15 |    |    |    |
| Paraffin oil.....                      |    |    |    | 20 |    |    |    |    |    |    |    | 15 |
| Santo resin (Standard) (Monsanto)..... | 15 | 20 | 20 | 15 | 35 | 15 | 25 |    | 20 | 20 | 20 |    |
| Santo resin 13.813, M. P. 84° C.....   |    |    |    |    |    | 30 |    | 30 |    |    |    |    |
| Santo resin B-53, M. P. 122° C.....    |    |    |    |    |    |    |    |    |    |    |    | 15 |
| Vistanex.....                          |    |    |    |    |    |    |    |    |    | 5  |    |    |
| Paraffin wax, M. P. 180° F.....        |    |    |    |    |    |    |    |    | 40 |    |    |    |
| Paraffin wax, M. P. 155° F.....        |    |    |    |    |    |    |    |    |    | 55 |    |    |
| Paraffin wax, M. P. 125° F.....        |    |    |    |    |    |    |    |    |    |    | 70 | 40 |
| Carnauba wax.....                      | 60 | 50 | 55 | 65 | 35 | 35 | 45 | 40 | 20 |    | 10 | 30 |
| Stearic acid.....                      |    |    |    |    |    |    | 10 | 15 |    |    |    |    |
| Hydrogenated castor oil.....           |    |    |    |    |    |    |    |    |    | 10 |    |    |

Other suitable formulae including other resins than Santo resins are given in Table II:

TABLE II  
*Percentage composition*

|                             | 13 | 14 | 15 | 16 | 17 | 18 | 19 | 20 | 21 | 22 | 23 | 24 |
|-----------------------------|----|----|----|----|----|----|----|----|----|----|----|----|
| Soya bean oil               |    |    |    |    | 10 | 10 | 10 |    |    |    |    |    |
| Castor oil                  |    |    |    |    |    |    |    |    |    | 10 | 16 | 15 |
| Cumar DX                    |    |    |    |    | 30 |    |    |    |    |    |    |    |
| Cumar RS                    |    |    |    |    |    | 30 |    |    |    |    |    |    |
| Neville R-10 Hard           |    |    |    |    |    |    | 30 |    |    |    |    |    |
| Neville R-15 Medium         |    |    |    |    |    |    |    | 30 |    |    | 20 |    |
| Vistanex                    |    |    |    |    |    |    |    |    | 10 |    | 5  |    |
| Paraffin wax, M. P. 155° F. |    |    |    |    | 60 | 60 | 60 |    |    | 60 | 80 | 60 |

oleaginous materials of the transfer composition may be incorporated if desired, although it is not essential when the transfer sheet is to be used to produce impressions which are to be reinked.

Pigments, preferably, should not be used since they tend to interrupt the continuity of the resin wax phase, but if used in small amounts, for example, not more than 5 to 10 per cent and milled

The transfer sheets of this invention are particularly suitable for the production of master copies which may be reinked and used in the production of thousands of copies. In this process a thin aluminum sheet having a surface to which water and the transfer composition will both adhere is assembled with the transfer sheet as shown in Fig. 1 and negative impressions

produced on the back of the aluminum sheet 3 by the keys 4 of a typewriter striking against the front of the aluminum plate backed by the transfer sheet. The aluminum plate containing the negative impression is removed from the typewriter, moistened with water and inked. The water adheres to the surface of the aluminum plate but does not adhere to the negative impression because the negative impressions are composed mainly of materials which are water repellent. The ink adheres to the negative impression but not to the surface of the plate containing the protective film of water, because the ink is made of a dye carrying composition such as the transfer composition of this invention which is water repellent, but adherent to itself. The metal sheet carrying the inked negative impressions is then contacted with sheets of paper 5 or the like thereby producing positive copies. By contacting the metal master with an inking and moistening device, followed by copy sheets, there may be produced thousands of clear and distinct copies.

Although the transfer composition and transfer sheets of this invention are particularly suitable for producing adherent impressions on grained or otherwise prepared water adherent surfaces, metal or otherwise, it is not restricted to such use, but may be used any place where strongly adherent, water repellent impressions are desired.

While there have been shown and described certain forms of the invention, it is to be understood that it is capable of many modifications. Changes, therefore, may be made without departing from the spirit and scope of the invention as described in the appended claims, in which it is the intention to claim all novelty inherent in the invention as broadly as possible, in view of the prior art.

The term "oleaginous" is used in the specification to mean oily and waxy materials of a water repellent nature such as soya bean oil, paraffin oil, paraffin waxes, undecylenic acid, castor oil, and the like.

We claim:

1. A transfer sheet adapted for use with pressure or impact instrumentalities in the production of impressions on master sheets for planographic printing, comprising a base sheet having a coating thereon of a transfer composition which is water-repellent, oil-ink absorbent, and transferable by pressure without heat to a contacting sheet, said transfer composition comprising soya bean oil, a carnauba wax which is compatible with the soya bean oil and modifies the mechanical properties thereof, and a hydrocarbon resin obtained by the treatment of an unsaturated petroleum fraction by a Friedel-Crafts catalyst.

2. A transfer sheet adapted for use with pressure or impact instrumentalities in the production of impressions on master sheets for planographic printing, comprising a base sheet having a coating thereon of a transfer composition which is water-repellent, oil-ink absorbent, and transferable by pressure without heat to a

contacting sheet, said transfer composition comprising oleaginous material and, as an agent for promoting adhesion of the composition to a master or like sheet, a hydrocarbon resin obtained by the treatment of an unsaturated petroleum fraction by a Friedel-Crafts catalyst, compatible with said oleaginous material.

3. A transfer sheet adapted for use with pressure or impact instrumentalities in the production of impressions on master sheets for planographic printing, comprising a base sheet having a coating thereon of a transfer composition which is water-repellent, oil-ink absorbent, and transferable by pressure without heat to a contacting sheet, said transfer composition comprising paraffin wax and, as an agent for promoting adhesion of the composition to a master or like sheet, a hydrocarbon resin obtained by the treatment of an unsaturated petroleum fraction by a Friedel-Crafts catalyst, compatible with said oleaginous material.

4. A transfer sheet adapted for use with pressure or impact instrumentalities in the production of impressions on master sheets for planographic printing, comprising a base sheet having a coating thereon of a transfer composition which is water repellent, oil-ink absorbent, and transferable by pressure without heat to a contacting sheet, said transfer composition comprising soya bean oil and, as an agent for promoting adhesion of the composition to a master or like sheet, a hydrocarbon resin obtained by the treatment of an unsaturated petroleum fraction by a Friedel-Crafts catalyst, compatible with said soya bean oil.

5. A transfer sheet adapted for use with pressure or impact in the production of impressions on master sheets for planographic printing, comprising a base sheet of paper having a coating thereon of a composition which is water repellent, oil-ink absorbent and transferable to a metal master sheet by the application of pressure or impact without heat, and which on the master sheet is capable of being inked, contacted directly with copy sheets and re-inked a plurality of times, said composition being composed essentially of paraffin wax and from 10 to 50% of a hydrocarbon resin which is compatible with said paraffin wax.

6. A transfer sheet adapted for use with pressure or impact in the production of impressions on master sheets for planographic printing, comprising a base sheet of paper having a coating thereon of a composition which is water repellent, oil-ink absorbent and transferable to a metal master sheet by the application of pressure or impact without heat, and which on the master sheet is capable of being inked, contacted directly with copy sheets and re-inked a plurality of times, said composition being composed essentially of paraffin wax, carnauba wax, and from 10 to 50% of a hydrocarbon resin obtained by the treatment of an unsaturated petroleum fraction with a Friedel-Crafts catalyst.

JOHAN BJORKSTEN.  
WILLIAM J. CHAMPION.